

## UNITED STATES PATENT OFFICE

1,955,796

## TREATMENT OF TEXTILE OR OTHER MATERIALS

George Holland Ellis, Spondon, near Derby, England, assignor to Celanese Corporation of America, a corporation of Delaware

No Drawing. Application November 26, 1930,  
Serial No. 498,436. In Great Britain January  
2, 1930

## 22 Claims. (Cl. 8—5)

This invention relates to the treatment of textile or other materials.

In the colouration of materials e. g. yarns, threads, fabrics or films, difficulty often occurs owing to the fact that dyestuffs and reagents may not readily penetrate the materials. This difficulty applies in particular to materials, such as those made of or containing cellulose derivatives, which exhibit a low degree of water absorption. An operation in which a ready penetration of a reagent into a material is especially important is the printing of materials, and the difficulty arising from lack of easy penetration is particularly noticeable in printing with white or coloured discharge pastes. In the case of these printing operations attempts have been made to get over the difficulty by adding certain hydroxy bodies such as alcohol, phenol, or resorcinol to the printing paste, and improved results have been obtained.

It has now been found that para-dihydroxy compounds, especially those of the benzene series, or derivatives of these compounds are exceedingly valuable agents for aiding the penetration of dyestuffs and other reagents into textile and other materials. They have been found of especial value for use in preparations for the local application of colouring matters or discharges to materials made of or containing cellulose derivatives.

According to the present invention therefore, para-dihydroxy compounds and derivatives of para-dihydroxy compounds are employed as aids to penetration of colouring matters, discharges, or other reagents into textile and other materials, and especially into materials made of or containing cellulose derivatives.

As examples of compounds which may be employed in accordance with this invention, hydroquinone, 2:5 dihydroxy-toluene, and their mono alkyl or aryl ethers or halogen derivatives may be mentioned. Any other desired assistants may be used, for example, anthraquinone or alcohol in printing. As has been stated, while these para-dihydroxy compounds may be employed in assisting penetration of the dyestuff, when dyeing in a dye bath, they are especially valuable in the local application of colouring matter or discharges, more particularly in the production of white and coloured discharge or discharge resist effects. The discharges or discharge resists may be oxidation discharges, for example chlorate discharges, or reduction discharges, e. g. hydrosulphite or sulphoxylate discharges.

After printing or stenciling with the paste or preparation containing the para-dihydroxy compound or derivative thereof drying may follow and the printed or stencilled materials may then

be suitably aged or steamed, or further rinsed, soaped, and finished as desired.

The following examples, while in no way limiting the invention, illustrate the best methods known to us for carrying the invention into effect:—

65

## Example 1

A cellulose acetate fabric dyed golden yellow by means of the dyestuff 4-chlor-2-nitro-4'-methoxy-diphenylamine is printed with a paste having the following composition:—

|                      | Parts by weight |
|----------------------|-----------------|
| Hydron pink FF paste | 15              |
| Gum arabic 1/1       | 50 75           |
| Water                | 12              |
| Hydroquinone         | 1               |
| Caustic soda         | 2               |
| Hydrosulphite powder | 3               |
| Anthraquinone        | 2 80            |
| Methylated spirits   | 5               |
| Formosul             | 10              |

The fabric is then dried and aged until the requisite degree of discharge is obtained, after which it is washed and subjected to an after-treatment for the oxidation of the vat colour.

85

## Example 2

A cellulose acetate fabric is dyed a medium shade of blue by first applying ortho-ethoxy-benzene-azo- $\alpha$ -naphthylamine and then diazotizing and developing on the fibre with  $\beta$ -oxynaphthoic acid. It is then prepared for printing as required and printed with a paste having the following composition:—

|                           | Parts by weight |
|---------------------------|-----------------|
| Hydron orange R. F. paste | 15              |
| Gum arabic 1/1            | 50 100          |
| Water                     | 12              |
| Hydroquinone              | 1               |
| Caustic soda              | 2               |
| Hydrosulphite powder      | 3               |
| Methylated spirits        | 5 105           |
| Anthraquinone             | 2               |
| Formosul                  | 10              |

The fabric is then dried and aged until the requisite degree of discharge is obtained.

110

## Example 3

A cellulose acetate fabric is dyed a dull green by means of a mixture of 4-chlor-2-nitro-4'-methoxy-diphenylamine and the compound obtained by coupling diazotized 2:4-dinitro-6-methoxy-1-amino-benzene with the product of

115

the condensation of epichlorhydrin and  $\alpha$ -naphthylamine. It is then prepared for printing and printed with a paste having the following composition:—

|                                        | Parts by<br>weight |
|----------------------------------------|--------------------|
| Ciba scarlet G (Colour Index No. 1228) | 15                 |
| Gum arabic 1/1                         | 50                 |
| Water                                  | 12                 |
| 10 Hydroquinone                        | 1                  |
| Caustic soda                           | 2                  |
| Hydrosulphite powder                   | 3                  |
| Methylated spirits                     | 5                  |
| Anthraquinone                          | 2                  |
| 15 Formosol                            | 10                 |

The fabric is then dried and aged until the requisite degree of discharge has been obtained.

While the invention has been described above more particularly with reference to the production of local colourations on cellulose acetate materials, it is also of great value in the treatment of materials containing other cellulose esters, e. g. cellulose formate, cellulose propionate, and cellulose butyrate, or containing cellulose ethers, for example methyl cellulose, ethyl cellulose and benzyl cellulose; and of materials containing cellulose derivatives in association with other fibres. It may also be usefully applied to the treatment of material containing other fibres than derivatives of cellulose, e. g. materials containing natural silk.

What I claim and desire to secure by Letters Patent is:—

- 35 1. In the treatment of materials, improving the penetration of reagents by means of a compound of the benzene series having two groupings of the type OX in para position to each other, where X is hydrogen, an alkyl, or an aryl grouping.
- 40 2. In the colouration of materials improving the penetration of reagents by means of a compound of the benzene series having two groupings of the type OX in para position to each other, where X is hydrogen, an alkyl, or an aryl grouping.
- 45 3. In the colouration of materials comprising a cellulose derivative, improving the penetration of reagents by means of a compound of the benzene series having two groupings of the type OX in para position to each other, where X is hydrogen, an alkyl, or an aryl grouping.
- 50 4. In the colouration of materials comprising cellulose acetate, improving the penetration of reagents by means of a compound of the benzene series having two groupings of the type OX in para position to each other, where X is hydrogen, an alkyl, or an aryl grouping.
- 55 5. In the colouration of materials comprising a cellulose derivative, improving the penetration of reagents by means of a para-dihydroxy body of the benzene series.
- 60 6. In the colouration of materials comprising cellulose acetate, improving the penetration of reagents by means of a para-dihydroxy body of the benzene series.
- 65 7. Process for printing materials comprising a cellulose derivative, characterized in that the material is printed with a printing preparation containing a compound of the benzene series having two groupings of the type OX in para position to each other, where X is hydrogen, an alkyl, or an aryl grouping.
- 70 8. Process for printing materials comprising cellulose acetate, characterized in that the material is printed with a printing preparation con-

taining a compound of the benzene series having two groupings of the type OX in para position to each other, where X is hydrogen, an alkyl, or an aryl grouping.

9. Process for printing materials comprising a cellulose derivative, characterized in that the material is printed with a printing preparation containing a para-dihydroxy body of the benzene series.

10. Process for printing materials comprising cellulose acetate, characterized in that the material is printed with a printing preparation containing a para-dihydroxy body of the benzene series.

11. Process for printing materials comprising a cellulose derivative, characterized in that the material is printed with a printing preparation containing hydroquinone.

12. Process for printing materials comprising cellulose acetate, characterized in that the material is printed with a printing preparation containing hydroquinone.

13. Process for producing discharge effects on materials comprising a cellulose derivative, characterised in that the material is printed with a discharge containing a compound of the benzene series having two groupings of the type OX in para position to each other, where X is hydrogen, an alkyl or an aryl grouping.

14. Process for producing discharge effects on materials comprising cellulose acetate, characterised in that the material is printed with a discharge containing a compound of the benzene series having two groupings of the type OX in para position to each other, where X is hydrogen, an alkyl, or an aryl grouping.

15. Process for producing discharge effects on materials comprising a cellulose derivative, characterised in that the material is printed with a discharge preparation containing a para-dihydroxy body of the benzene series.

16. Process for producing discharge effects on materials comprising cellulose acetate, characterised in that the material is printed with a discharge preparation containing a para-dihydroxy body of the benzene series.

17. Process for producing discharge effects on materials comprising a cellulose derivative, characterised in that the material is printed with a discharge preparation containing hydroquinone.

18. Process for producing discharge effects on materials comprising cellulose acetate, characterised in that the material is printed with a discharge preparation containing hydroquinone.

19. In the treatment of materials comprising a cellulose derivative, improving the penetration of reagents by means of a compound of the benzene series having two groupings of the type OX in para position to each other, where X is hydrogen, an alkyl, or an aryl grouping.

20. In the treatment of materials comprising cellulose acetate, improving the penetration of reagents by means of a compound of the benzene series having two groupings of the type OX in para position to each other, where X is hydrogen, an alkyl, or an aryl grouping.

21. In the treatment of materials comprising a cellulose derivative, improving the penetration of reagents by means of a para-dihydroxy body of the benzene series.

22. In the treatment of materials comprising cellulose acetate, improving the penetration of reagents by means of a para-dihydroxy body of the benzene series.